# EUROPEAN PATENT SPECIFICATION

(11) **EP 0 162 930 B1**
(45) Date of publication and mention of the grant of the patent: **22.08.1990**
(21) Application number: 84904178.5
(22) Date of filing: 22.11.1984
(51) Int. Cl.: B41M 5/035

(54) **IMAGE-RECEIVING MATERIAL**
BILDEMPFANGSMATERIAL
MATERIAU RECEPTEUR D'IMAGES

(30) Priority: 24.11.1983 JP 221047/83
(43) Date of publication of application: 04.12.1985
(73) Proprietor: MATSUSHITA ELECTRIC INDUSTRIAL CO., LTD., Kadoma-shi, Osaka-fu, 571 (JP)
(72) Inventor: TAKASHIMA, Yuji, Nishinomiya-shi Hyogo-ken 662 (JP); YUBAKAMI, Keiichi, Suita-shi, Osaka-fu 565 (JP); SHIMIZU, Tokihiko, Ikoma-gun Nara-ken 636-01 (JP)
(74) Representative: Patentanwälte Leinweber & Zimmermann
(86) International application number: JP8400559
(87) International publication number: WO8502375

(56) References cited:
- DE-A- 3 237 381
- DE-A- 3 303 427
- JP-A- 5 232 716
- JP-A- 5 348 751
- JP-A- 5 816 885
- JP-A-49 111 711
- US-A- 3 870 435
- US-A- 4 089 547
- PATENT ABSTRACTS OF JAPAN, vol. 7, no. 193 (M-238)[1338], 24th August 1983; & JP-A-58 94 491 (MITSUBISHI SEISHI K.K.) 04-06-1983
- PATENT ABSTRACTS OF JAPAN, vol. 7, no. 165 (M-230)[1310], 20th July 1983; & JP-A-58 72 495 (JIYUUJIYOU SEISHI K.K.) 30-04-1983
- PATENT ABSTRACTS OF JAPAN, vol. 7, no. 92 (M-208)[1237], 16th April 1983; & JP-A-58 16 884 (CANON K.K.) 31-01-1983
- CHEMICAL ABSTRACTS, vol. 96, no. 24, June 1982, page 606, abstract no. 208425g, Columbus, Ohio, US; & JP-A- 81 148 583 (CANON K.K.) 18-11-1981
- PATENT ABSTRACTS OF JAPAN, vol. 7, no. 227 (M-248)[1372], 7th October 1983; & JP-A-58 119 888 (CANON K.K.) 16-07-1983
- PATENT ABSTRACTS OF JAPAN, vol. 6, no. 263 (M-181)[1141], 22nd December 1982; & JP-A-57 157 786 (MITSUBISHI SEISHI K.K.) 29-09-1982
- PATENT ABSTRACTS OF JAPAN, vol. 6, no. 33 (M-114)[911], 27th February 1982; & JP-A-56 148 586 (CANON K.K.) 18-11-1981
- PATENT ABSTRACTS OF JAPAN, vol. 4, no. 94 (M-19)[576], 8th July 1980; & JP-A-55 51 583 (RICOH K.K.) 15-04-1980

## Description

The invention relates to an image receptor having a structure in which a color forming layer causing color development of a sublimable dye which develops color when adsorbed by an electron-acceptant material is provided on a substrate.

A variety of image recording methods using only a dye material itself as inking material have been proposed hitherto. For instance, there are known a one-shot electrophotographic method using light transmitting particles containing a subliming color former as disclosed in Japanese Patent Publication No. 49307/80; a sublimation transfer method in which a color sheet prepared by coating a condenser paper or the like with a subliming dye is heated by a heating element so that the sublimed dye develops color on an image receptor; and a gas jet recording method disclosed in Japanese Patent Publication No. 2020/81 in which gas of a subliming dye is electrically injected and controlled to obtain a dye image on an image receptor.

In any of the above-described methods, it is necessary to let the dye develop color in a molecular state and uniformly on an image receptor for obtaining a clear dye image. For this purpose, there is usually used an image receptor carrying a dye developer. In the prior art, bottom paper for pressure-sensitive recording using activated clay as color developer has been used for said image receptor.

Such bottom paper, however, had the problem of reduced color purity of the dye image for such reasons that (1) activated clay is tinted in light brown, and (2) the color-forming layer becomes opaque because of poor transparency of activated clay. Therefore, said bottom paper was not suitable for color recording especially.

Another type of recording is inkjet recording, and an image receptor for ink jet recording is disclosed in DE-A-3 237 381. In this method droplets of a liquid recording ink are applied to the image receptor in accordance with a desired recording pattern. In order to firmly adhere the recorded pattern of ink droplets to the image receptor and to avoid excessive blot of the ink droplets, the recording surface of the image receptor has coated thereon a porous layer exhibiting a high absorption rate for the recording ink. Various materials may be selected for this absorptive layer and a binder used therewith, these materials including silicon dioxide particles of a certain size and styrene-butadiene copolymer as the binder.

In a still other method used for the transfer of color from one sheet to another in a manifold paper system by the impact of a type or by the pressure of a pen or pencil, use is made of fumed hydrophilic silicon dioxide particles adhered to the receptor sheets. This will allow for thinner and lighter sheets resulting in a reduced pressure for writing to allow for more accurate replication and a greater number of copies.

The object of this invention is to provide an image receptor of the above-referenced type used for image recording employing only a sublimable dye material itself as inking material, in which the color-forming layer containing color developer is improved in heat resistance and transparency.

In accordance with the invention this object is attained in that said color forming layer contains both silicon dioxide as main color developer of said sublimable dye and a styrene-butadiene copolymer as a binder of said silicon dioxide.

The color-forming layer has the function to let the dye develop color in a molecular state and uniformly. It is of improved gas permeability for the subliming dye and of improved heat resistance. Thereby a clear and highly transparent color image can be obtained.

### Brief Description of the Drawing

The drawing is a schematic sectional view showing an embodiment of image receptor in accordance with this invention.

### Best Mode for Carrying out the Invention

In an embodiment of image receptor in accordance with this invention, a color-forming layer 3 principally composed of silicon dioxide 2 is carried on a substrate 1 as illustrated in the drawing.

Silicon dioxide 2 is used as color developer and has excellent transparency. It is colorless and suffers from no thermal yellowing because of heat resistance, making it possible to obtain a dye image with high color purity. As silicon dioxide used in this invention, there can be employed amorphous, glassy or colloidal silicon dioxide. Among them, colloidal silicon dioxide with a pH of 6 or below is especially excellent as it has the excellent ability to cause color development of dye and that the color forming layer can be easily made transparent.

For substrate 1, various types of substrate material can be applied according to the purpose of use. For instance, fine-quality paper or art paper with high whiteness is suited for reflective pictures such as documents. Plastic sheet with excellent transparency and heat resistance such as vinylon, cellophane, acetyl-cellulose or the like is suited for transmitting pictures such as slides.

Color forming layer 3 can be made transparent by coating silicon dioxide finely dispersed in a binder on substrate 1 by a usual means such as bar coater. In this case, the particle size of silicon dioxide is preferably not greater than 0.1 micron.

The binder is preferably one which is strong in binding force, transparent and also excellent in silicon dioxide dispersability. A combination of styrene-butadiene copolymer and colloidal silicon dioxide is especially suited for the applications where the image receptor is heated since such combination is hardened and improved in heat resistance when heated.

For attaining better color developing efficiency of the dye, it is preferred to make the color forming layer porous so that the dye becomes more easily absorbed by silicon dioxide. For this purpose, it is desirable that the amount of the binder used is not greater than 30% by weight based on silicon dioxide. The coating weight of the color forming layer for effecting sufficient color development of the dye is preferably 1-10 g/m² although is it variable depending on the type of the dye used.

It is of course possible, where necessary, to add a dispersant when dispersing silicon dioxide in binder or to add an anti-oxidant or a quencher to the color forming layer for the purpose of preventing color fading of the dye. Further, an electron acceptant material such as a known organic or inorganic acid may be used jointly with silicon dioxide as a color developing assistant.

### Example 1

The following materials were well stirred and mixed by a mixer to form a color forming layer solution.

### Color developer:

This color forming layer solution was coated on a sheet of art paper to a coating weight (after drying) of 6 g/m² to obtain an image receptor A for reflective picture.

### Example 2

The color forming layer solution of Example 1 was coated on a vinylon sheet to a coating weight of 6 g/ m² to obtain an image receptor B for transmitting picture. Transmittance of the image receptor was 90%.

### Comparative Example 1

A mixture of the following formulation was sufficiently dispersed by an attritor to prepare a color forming layer solution.

### Color developer:

This color forming layer solution was coated on a fine-quality paper to a coating weight (after drying) of 8 g/m² to obtain an image receptor C for reflective picture.

### Experiment 1

A yellow disperse dye ("PT-52Y" produced by Mitsubishi Kasei Kogyo KK), a mangenta basic dye (C.I. Basic Red 9) and a magenta subliming color former (7'-diethylamino-1,3,3,5-tetramethyl-indolino- benzospiropyran) were coated on a 15 micron thick condenser paper by using ethyl cellulose as binder to prepare three types of color sheets D, E and F. The image receptor obtained in the Examples and Comparative Example and said color sheets were placed one upon the other and heated under the conditions of 180°C, 5 seconds and 1 kg/cm², whereby the distinct yellow and magenta color images such as shown in Table 1 were obtained on the image receptor. The numerical figures in the table indicate color density.

### Experiment 2

Color sheet F was superposed on the yellow color images obtained by using color sheet D in Experiment 1, and heated under the same conditions as Experiment 1, whereby the distinct red color images such as shown in Table 2 were obtained.

### Industrial Applicability

The image receptor of this invention can make the color forming layer transparent as silicon dioxide with excellent transparency is used as color developer. Therefore, there is no possiblity that the dye which developed color below the color forming layer be concealed by the color developer thereabove to reduce the developed color density, and the whole color forming layer becomes a colored transparent body, so that a dye image with high developed color density can be obtained, enabling realization of high-quality pictures by electrophotography or printers.

## Claims

1. An image receptor having a structure in which a color forming layer (3) causing color development of a sublimable dye which develops color when adsorbed by an electron-acceptant material is provided on a substrate (1), characterized in that said color forming layer (3) contains both silicon dioxide (2) as main color developer of said sublimable dye and a styrene-butadiene copolymer as a binder of said silicon dioxide (2).

2. An image receptor according to Claim 1, wherein the amount of the styrene-butadiene copolymer is 30% by weight or less based on silicon dioxide (2).

3. An image receptor according to Claim 1 or 2, wherein silicon dioxide (2) is a solidified material of colloidal silicon dioxide having a pH of 6 or below.

4. An image receptor according to any one of Claims 1 to 3, wherein the substrate (1) is paper.

5. An image receptor according to any one of Claims 1 to 3, wherein the substrate (1) is a transparent plastic film.

## Patentansprüche

1. Bildaufnehmer mit einem Aufbau, bei dem eine farbbildende Schicht (3), die eine Farbentwicklung eines sublimierbaren Farbstoffes, der bei Adsorption durch ein elektronenaufnehmendes Material Farbe entwickelt, hervorurruft, auf einem Substrat (1) vorgesehen ist, dadurch gekennzeichnet, daß die farbbildende Schicht (3) sowohl Siliziumdioxid (2) als Hauptfarbentwickler des sublimierbaren Farbstoffs als auch Styrolbutadienkopolymer als ein Bindemittel für das Siliziumdioxid (2) enthält.

2. Bildaufnehmer nach Anspruch 1, bei dem die Menge an Styrolbutadienkopolymer 30 Gewichtsprozent oder weniger bezogen auf Siliziumdioxid (2) ist.

3. Bildaufnehmer nach Anspruch 1 oder 2, bei dem das Siliziumdioxid (2) ein verfestigtes Material aus kolloidalem Siliziumdioxid mit einem pH von 6 oder darunter ist.

4. Bildaufnehmer nach einem der Ansprüche 1 bis 3, bei dem das Substrat (1) Papier ist.

5. Bildaufnehmer nach einem der Ansprüche 1 bis 3, bei dem Substrat (1) eine transparente Kunststoffolie ist.

## Revendications

1. Récepteur d'image ayant une structure dans laquelle une couche formatrice d'image (3) produisant le développement en couleur d'un colorant sublimable qui développe une couleur lorsqu'il est adsorbé par un accepteur d'électrons est disposée sur un substrat (1), caractérisé en ce que ladite couche formatrice de couleur (3) contient à la fois du bioxyde de silicium (2) en tant que développateur de couleur principal dudit colorant sublimable et un copolymère styrène/butadiène en tant que liant de ce bioxyde de silicium (2).

2. Récepteur d'image selon la revendication 1, dans lequel la proportion du copolymère styrènel butadiène est de 30% en poids ou moins sur la base du bioxyde de silicium (2).

3. Récepteur d'image selon la revendication 1 ou 2, dans lequel le bioxyde de silicium (2) est un matériau provenant de la solidification de bioxyde de silicium colloïdal, ayant un pH de 6 ou au-dessous.

4. Récepteur d'image selon l'une quelconque des revendications 1 à 3, dans lequel le substrat (1) est du papier.

5. Récepteur d'image selon l'une quelconque des revendications 1 à 3, dans lequel le substrat (1) est un film de matière plastique transparente.
